

Sept. 27, 1960

O. OSBORN ET AL  
ALKALINE HYDROXIDES IN CATHODIC PROTECTION  
OF METALS IN SEAWATER AND BRINES  
Filed May 23, 1951

2,954,332



INVENTORS.  
Oliver Osborn  
BY John Joseph Newport<sup>III</sup>

Griswold & Burdick  
ATTORNEYS

# United States Patent Office

2,954,332

Patented Sept. 27, 1960

1

2,954,332

## ALKALINE HYDROXIDES IN CATHODIC PROTECTION OF METALS IN SEAWATER AND BRINES

Oliver Osborn, Lake Jackson, and John Joseph Newport III, Freeport, Tex., assignors to The Dow Chemical Company, Midland, Mich., a corporation of Delaware

Filed May 23, 1951, Ser. No. 227,906

6 Claims. (Cl. 204—56)

This invention relates to an improved method and system for the cathodic protection of metals in seawater and like brines.

It is well recognized that steel and other corrodible metals in contact with seawater can be protected against corrosion by applying electric current to the metal as cathode. If small currents are used, of the order of 0.005 to 0.01 ampere per square foot, the metal, while protected by the cathodic potential, remains largely bare; a solid cathodic coating may form on it after many months. On the other hand, with larger currents, e.g. over 0.03 ampere per square foot, a calcareous coating is produced and thoroughly covers the metal within a day or two, or even much less time, if a high enough current is used (cf. U.S. Patent 2,200,469). This coating appears to consist mainly of the carbonates and hydroxides of calcium and magnesium. Although slightly soluble in seawater, it will remain in place and afford considerable protection to the metal for a long time after all flow of current is ended. Further, the coating may be maintained intact at much lower current densities than are required to produce it. Optimum cathodic protection of metal in seawater, then, calls for intentional rapid production of the calcareous coating at high current, followed by the application of a lower maintenance current continuously. This latter procedure, though effective, has been expensive because of the high current requirements while the coating is being formed. If sufficient permanent capacity is installed to supply the initial current, most of that capacity remains unused for the duration of the protection period, often for years. On the other hand, the cost of acquiring and moving a portable high-current low-voltage generator, such as might be used as a booster in the initial stages of protection, has also proven excessive.

The present invention seeks to eliminate this source of expense by providing a method of forming the protective cathodic calcareous coatings on metals without supplying the high initial currents heretofore required. It also provides a method of forming and maintaining such coatings at far lower current densities than have been possible previously.

These results are realized according to the invention by adding to the seawater or other like brine in contact with the metal to be protected a water-soluble alkaline hydroxide in an approximate proportion of from 2 parts to 300 parts per million. With the water thus alkalized, formation of a protective calcareous coating occurs at current densities as little as a tenth of those required when the alkalinity is absent. The current density needed to maintain the coating is also reduced, though not quite as much.

So far as known, the new process is applicable in the cathodic protection not only of iron and steel, but also of all other corrodible metals no more anodic than zinc. It is effective in preventing corrosion both by seawater and by other saline brines containing both calcium and magnesium salts in substantial proportion. Typical

2

of these latter are the diluted seawater found in many ports, and the inland brines of Michigan and Ohio, which are probably concentrates of the water of ancient seas.

The water-soluble alkaline hydroxides used in the invention should be strongly basic. Sodium hydroxide appears to be most satisfactory and usually also the cheapest. However, other soluble basic hydroxides, especially calcium hydroxide, aqueous ammonia, and the hydroxides of potassium, barium, and strontium may be used where available. The hydroxide may be added in solid form or in aqueous solution, either concentrated or dilute. Since the purity of the hydroxide is of no great moment, it is usually most economical, where possible, to use waste alkaline hydroxide-containing process liquors, which may be quite dilute, such as effluent catholyte from electrolytic brine cells, caustic soda evaporator tail water, spent caustic liquor from organic chemical reactions, and the like.

The proportion of alkaline hydroxide according to the invention falls in the approximate range of 2 parts to 300 parts per million. At even as little as 2 parts per million, very substantial savings in current can be realized in forming a calcareous coating on steel in seawater. At much over 300 parts per million, alkali is consumed to no purpose. Preferred concentrations, in the case of sodium hydroxide, are in the range of 25 to 50 parts per million when a cathodic coating is to be formed rapidly, and from 2 to 10 parts per million when it is to be produced more slowly, or when a coating already formed is to be maintained.

The current densities required for coating formation according to the invention depend in some measure on the concentration of alkali added to the seawater or other brines, and also on the salinity of the brine. In all cases, however, they are lower than those required in the absence of the alkali. For instance, in seawater to which 25 to 50 parts per million of sodium hydroxide is added, a current density not over 0.02 ampere per square foot is adequate for formation of the protective calcareous coating in a reasonably short time, usually less than a month, and often with a few days or less. If rapidity of coating formation is not important, adequate cathodic protection can be realized at a sodium hydroxide concentration of 2 to 10 parts per million and at a current density of from 0.002 to 0.005 ampere per square foot. A coating may form slowly over a period of several months. These latter conditions will also suffice to maintain an existing cathodic calcareous coating.

The process of the invention is extremely useful in connection with steel and other metal vessels for storing seawater and brines, and the similar tanks aboard tanker ships, where seawater is sometimes used for ballast. In such cases, only a single addition of sodium hydroxide is required for each filling of the tank. Another use is in the cathodic protection of flumes, pipelines, condenser jackets and other conduits through which seawater is made to flow. In these instances, the alkali must be continuously added to the seawater, preferably at or ahead of its point of entry into the conduit.

In the invention, the requisite current for rendering cathodic the metal to be protected may be generated in any of the usual ways. However, the use of sacrificial anodes, particularly those made of magnesium or magnesium-base alloys (hereinafter collectively termed magnesium metal) is eminently satisfactory. Magnesium has the advantage that its self-generated potential is sufficient to insure adequate cathodic protection but is not sufficient to cause excessive electrolysis. Hence, with magnesium anodes, there is automatically supplied a current which is only slightly in excess of the minimum required for adequate protection.

The invention, in one preferred embodiment, may be explained with reference to the accompanying schematic drawing. In the system there shown, a large bare steel pipeline 1 is being used for carrying flowing seawater, only a small portion of the line being shown. A covered manhole 2 is provided for access to the interior of the pipe 1. Within the pipe, sacrificial magnesium anodes 3 are placed at intervals, being suspended on electrically conducting cables 4 which are welded to the pipe at one end and at the other are firmly connected to the magnesium. Near the inlet of the pipe 1 is a tank 5 for storing sodium hydroxide solution, the tank being connected to the pipe by a valved line 6. In operation, the line 6 acts as a continuous feeder of sodium hydroxide solution, the valve being adjusted to maintain the desired concentration of sodium hydroxide in the flowing seawater. The choice of the size and spacing of the magnesium anodes to afford the desired current density is according to well known principles.

The following examples will also illustrate the invention.

*Example 1*

In the system shown in the drawing, the inside surface of a 30-inch bare steel pipeline was protected against corrosion in seawater by sacrificial magnesium anodes each weighing 17 pounds, the anodes being spaced at 5-foot intervals. Recording ammeters were used to follow the current demands of the line. The rate of seawater flow was 100 gallons per minute.

For experimental purposes, weak sodium hydroxide solution was injected continuously into the pipeline part way along its length. In this manner, the first portion of the line was cathodically protected in ordinary seawater while the latter half was protected in alkalized seawater. The proportion of sodium hydroxide was regulated at 250 parts per million of seawater. Over a period of 26 days, the first part of the line drew current at a rate declining gradually from 0.045 to 0.033 ampere per square foot. No appreciable calcareous coating formed. The last part of the line drew current at a rate declining gradually from 0.020 to 0.010 ampere per square foot. A significant calcareous coating was formed.

As the experiment showed, the effect of the sodium hydroxide addition was to lower the current requirement of the line to about one-third of that called for in the absence of the hydroxide, and also to increase the rate at which a calcareous coating formed.

*Example 2*

The walls of a large flume carrying seawater at a velocity of a few feet per second are constructed of bare corrugated sheet-steel piling. A direct-current source was installed to supply current to the piling as cathode in an effort to protect it against corrosion. Over a period of several months, current was supplied at the maximum capacity of the source, corresponding to about 0.035 to 0.04 ampere per square foot of piling exposed to the seawater. Corrosion was reduced but complete protection was not achieved, and the structure never became fully polarized.

With the source still connected, aqueous sodium hydroxide was fed continuously into the flume near its mid-point longitudinally. The rate of addition corresponded to 2.5 parts per million of seawater. The portion upstream from the addition continued to draw current as before, with only partial protection being realized. However, downstream from the point of addition, it was found that complete protection and polarization could be realized with an ultimate current density of 0.002 ampere per square foot. Gradual formation of a calcareous coating took place over a period of several months.

The example shows that, with the addition of only 2.5 parts per million of sodium hydroxide, the current demand was reduced more than twenty-fold, at the same time providing better protection.

*Example 3*

In a laboratory demonstration, identical steel coupons having a surface area of 18.7 square inches were weighed and then subjected to corrosion testing. One group of 5 coupons were immersed in a vessel of seawater and current was supplied to the coupons as cathodes at a current density of 0.005 ampere per square foot for a period of 17 days. At the end of this time, the coupons were removed, cleaned of corrosion, and reweighed. Average 10 weight loss was about 1.15 gram.

In a parallel test, in which the seawater contained 50 parts per million of sodium hydroxide, after 17 days at 0.005 ampere per square foot, the average weight loss was about 0.29 gram. The addition of the sodium hydroxide to the seawater reduced the corrosion to one-fourth.

The electrochemical phenomena on which the invention is based are not fully understood. It is believed that the addition of the basic hydroxide to seawater or like brine induces precipitation of calcium carbonate in colloidal form. This precipitate may then become transferred by electrophoresis to the cathode being protected. There must be other factors at work, however, since the addition of sodium carbonate, for instance, will induce precipitation of calcium carbonate but will not enhance coating formation.

It is realized that in the conventional cathodic protection of steel in seawater, some small proportion of alkali may be generated at the steel surface by the electrolysis. However, the formation in situ of such hydroxide does not produce the results according to the invention, which requires the intentional addition of pre-existing basic hydroxide from an external source.

What is claimed is:

1. In a process wherein a corrodible metal no more anodic than zinc in contact with seawater is protected against corrosion by applying electric current to the metal as cathode to produce a calcareous coating thereon, the method of effecting such protection at minimum expenditure of electric energy which comprises the steps of dispersing a pre-existing water-soluble alkaline hydroxide throughout the seawater in an approximate proportion of from 2 parts to 300 parts per million and supplying current to the metal at an effective current density not exceeding 0.02 ampere per square foot and less than that required to produce a calcareous coating in the absence of added hydroxide.
2. A process according to claim 1 wherein the metal is steel, and the hydroxide is sodium hydroxide supplied in a proportion of 25 to 50 parts per million.
3. In a process wherein a steel conduit containing flowing seawater is protected against corrosion by applying electric current to the steel as cathode to produce a calcareous coating thereon, the method of effecting such protection at minimum expenditure of electric energy which comprises the steps of dispersing a pre-existing strongly basic hydroxide throughout the flowing seawater in a proportion between 2 parts and 300 parts per million prior to passage thereof through the conduit and supplying current to the steel at a current density not exceeding 0.02 ampere per square foot and less than that required to produce a calcareous coating in the absence of added hydroxide.
4. A method according to claim 3 wherein the hydroxide is sodium hydroxide.
5. A method according to claim 4 in which the hydroxide is added in an approximate proportion to 2 to 10 parts per million and the current is supplied at an approximate current density of from 0.002 to 0.005 ampere per square foot.
6. In a process wherein steel in contact with seawater is protected against corrosion by applying electric current to the steel as cathode to polarize the same, the method of effecting such protection at minimum expenditure of electric energy which comprises the steps of dispersing

pre-existing sodium hydroxide throughout the seawater in an approximate proportion of 2 to 10 parts per million while supplying current to the steel at a current density of from 0.002 to 0.005 ampere per square foot, such density being less than that required to produce polarization in the absence of added hydroxide.

References Cited in the file of this patent

UNITED STATES PATENTS

2,444,174 Tarr et al. ----- June 29, 1948 10  
2,534,234 Cox ----- Dec. 19, 1950

FOREIGN PATENTS

3,388 Great Britain ----- of 1903

OTHER REFERENCES

5 "Water Works and Sewerage," vol. 89 (1942), pages 285-291, article by O'Brien.

"Corrosion," vol. 2 (October 1946), pages 175 thru 187, article by Sudrabin.

"Corrosion," vol. 4 (July 1948), pages 358 thru 370, article by Humble.